

[54] **FROTH FLOTATION METHOD OF SEPARATING NAHCOLITE FROM ORES CONTAINING NAHCOLITE**

[75] Inventors: **Edward C. Rosar; Vuko M. Lepetic**, both of Lakewood; **John R. Hobaugh**, Denver, all of Colo.

[73] Assignee: **Industrial Resources, Inc.**, Chicago, Ill.

[22] Filed: **Oct. 18, 1971**

[21] Appl. No.: **190,416**

[52] U.S. Cl. .... **241/20**, 209/3, 209/164, 209/166

[51] Int. Cl. .... **B02c 21/00**

[58] Field of Search .... 209/166, 162, 160, 167, 209/164, 171; 241/20, 24

[56] **References Cited**

UNITED STATES PATENTS

|           |         |                |           |
|-----------|---------|----------------|-----------|
| 1,510,983 | 10/1924 | Dolbear .....  | 209/166 X |
| 2,762,509 | 9/1956  | Bachmann ..... | 209/166   |
| 2,937,751 | 5/1960  | Schoeld .....  | 209/166   |
| 3,525,434 | 8/1970  | Garrett .....  | 209/166   |

|           |         |                |           |
|-----------|---------|----------------|-----------|
| 2,175,178 | 10/1939 | Campbell ..... | 209/166   |
| 3,401,110 | 9/1968  | Floyd .....    | 209/166 X |
| 2,931,502 | 4/1960  | Schoeld .....  | 209/166 X |

FOREIGN PATENTS OR APPLICATIONS

|           |         |                     |         |
|-----------|---------|---------------------|---------|
| 18,601    | 8/1915  | Great Britain ..... | 209/162 |
| 446,418   | 4/1936  | Great Britain ..... | 209/166 |
| 669,100   | 7/1929  | France .....        | 209/160 |
| 834,833   | 2/1952  | Germany .....       | 209/166 |
| 838,059   | 12/1938 | France .....        | 209/166 |
| 1,185,522 | 1/1965  | Germany .....       | 209/166 |

OTHER PUBLICATIONS

Taggart, 1945, 12-125

Primary Examiner—Robert Halper  
Attorney, Agent, or Firm—Jacques M. Dulin

[57] **ABSTRACT**

A flotation method for the separation of Nahcolite from its crushed ores using a brine solution in equilibrium with the soluble components of the ore to selectively separate by flotation a concentrate of the Nahcolite from other ore constituents.

6 Claims, No Drawings

**FROTH FLOTATION METHOD OF SEPARATING  
NAHCOLITE FROM ORES CONTAINING  
NAHCOLITE**

Extensive dolomitic marlstone formations (called oil shales) exist throughout the western part of the United States, particularly the mountain states of Colorado, Utah, and Wyoming. Associated with certain sections of the shale beds is the mineral Nahcolite, which is a sodium bicarbonate. The Nahcolite mineral is quite soluble in aqueous solution. The shale is normally called oil shale, since it contains considerable amounts of an organic material referred to as kerogen which, on pyrolysis, produces a hydrocarbon type oil. The kerogen bearing rocks occur in beds, some of which exceed many hundreds of feet in thickness, and extraction of an oil from the shale has in the past been accomplished by a pyrolysis or a retorting process. The temperature of the retorting determines the type of product recovered.

Kerogen bearing rock in the Green River formation of the Piceance Creek Basin northwestern Colorado and extending into Utah and Wyoming, also, contains Gibbsite and Dawsonite along with Nahcolite. The oil shales extend in beds covering approximately 500 square miles and may occur through as much as 750 feet. Core drilling shows that Nahcolite may occur in a quantity from about 10 through 75 percent or even higher.

According to the present invention, a froth flotation concentration is provided for oil shale containing Nahcolite, in which ore is subjected to a flotation treatment to produce a concentrate of Nahcolite.

The froth flotation process is conducted in a brine in equilibrium with respect to the soluble constituents of the ore, that is, equilibrium at the temperature of the solution. The ore is reduced to particles of flotation size as required by its liberation characteristics.

Included among the objects and advantages of the present invention is to provide a froth flotation method of selectively separating Nahcolite from ores containing Nahcolite.

Another object of the invention is to provide a froth flotation process using an aqueous brine medium for the separation of Nahcolite from its ores.

Another object of the invention is to provide a froth flotation process for the separation of Nahcolite from oil shale containing Nahcolite and other soluble minerals.

A further object of the invention is to provide a froth flotation method for the separation of Nahcolite from its ores by inexpensive reagents and simplified methods.

Yet another object of the invention is to provide a froth flotation separation of Nahcolite from its ores in concentrated brine solution of the soluble constituents of the ore, which does not require high energy or high capital costs for the separation.

Another object of the invention is to provide a froth flotation separation of Nahcolite from Dawsonite and oil shale and as the result of it to upgrade the latter two simply and inexpensively before their further processing.

These and other objects and advantages of the invention will become apparent to those skilled in the art from consideration of the following description and claims.

The process of the present invention may utilize conventional froth flotation equipment and some known techniques. The collector reagents if any are necessary and other auxiliary reagents are chosen to produce a selective separation of the Nahcolite from the other ingredients in the ore, with the ore pulped in a brine of the soluble ingredients in the ore. The ore after having been mined is, of course, reduced to the flotation size as required for the liberation of Nahcolite. It is pulped in the brine as is conventional in the art.

The froth flotation of the present invention, using conventional equipment, may utilize standard procedures for a flotation treatment, wherein there may be scavenger flotation, a rougher flotation, a cleaner flotation or the like. By using various collector reagents, if any are necessary, the Nahcolite may be concentrated as the under flow, i.e. the non-float portion.

The ores which were tested assayed:

NaHCO<sub>3</sub>—from 45 to 57%

Na<sub>2</sub>CO<sub>3</sub>—from 1.0 to 1.5%

Oil—from 9 to 14 gal/ton

By x-ray diffraction the relative abundance of minerals was found to be:

Nahcolite (NaHCO<sub>3</sub>)—from 35 to 45%

Dolomite—from 15 to 30%

Analcime—from 20 to 25%

Quartz—from 10 to 15%

Feldspar—from 0 to 5%

A preliminary concentration of the Nahcolite is produced by a size reduction and a screening. The Nahcolite is more brittle than most of the rock ingredients, and it is reduced more than the others in a hammer mill. Screening the ground particles produces fines of a higher Nahcolite concentration than the original ore.

Size reduction, prior to a flotation beneficiation, is to liberate the desired values from its ore. In this case, the samples were crushed, in a hammer mill, to 100%-28 mesh (Tyler Screen). By screening of the crushed material assaying 56.9% NaHCO<sub>3</sub> the following results were shown:

| Screen Size | Weight % | Chemical Analysis% NaHCO <sub>3</sub> | Distribution% NaHCO <sub>3</sub> |
|-------------|----------|---------------------------------------|----------------------------------|
| +65m        | 19.2     | 25.1                                  | 8.4                              |
| -65m        | 80.8     | 65.1                                  | 91.6                             |

Screening at 100 mesh produces the following:

| Screen Size | Weight % | Chemical Analysis% NaHCO <sub>3</sub> | Distribution% NaHCO <sub>3</sub> |
|-------------|----------|---------------------------------------|----------------------------------|
| +100m       | 27.6     | 30.1                                  | 14.5                             |
| -100m       | 72.6     | 67.8                                  | 85.5                             |

This, of course, suggests the pre-concentration of Nahcolite by screening, prior to flotation. A phenomenon which occurs in a beneficiation process of the invention, is that kerogen in the ore is soft, and during the size reduction with certain types of size reduction equipment it generally smears over the associated inorganic materials. The smearing of course, prevents a clean separation of the organic and inorganic materials of the ore. It was found, however, that the use of a hammer mill for the size reduction tends to reduce the attendant smearing, and such equipment is one of the size reduction equipment of choice.

Laboratory tests were conducted on the crushed ore, by pulping the above samples with a brine in which the soluble ingredients of the ore are in equilibrium with soluble ingredients in the liquid. A Fagergren flotation machine was used for this investigation. Utilizing natural hydrocarbon coatings (which may have originated from the ore) on the gangue (non-Nahcolite) mineral particles and natural frothing of the brine, the gangue minerals were floated from Nahcolite without any flotation reagents. The following results were obtained from this test carried out on the feed preconcentrated

may improve the natural frothing characteristics of the brine or of the flotation pump itself.

Examples of the use of alcohols and also oil concentration in the float product are given below.

Conditioning Nahcolite - oil shale ore at the density of 25 percent solids with 1-Hexanol (4-5 lb/ton of flotation feed) an subsequently floating oil shale from Nahcolite would result in and substantial concentration of oil shale in the float product. The results of flotation tests conducted on three different ore samples were as follows:

| Weight (%)    | Chemical analysis (%) |                                 |                  | Distribution (%)   |                                 |                  |
|---------------|-----------------------|---------------------------------|------------------|--------------------|---------------------------------|------------------|
|               | NaHCO <sub>3</sub>    | Na <sub>2</sub> CO <sub>3</sub> | SiO <sub>2</sub> | NaHCO <sub>3</sub> | Na <sub>2</sub> CO <sub>3</sub> | SiO <sub>2</sub> |
| Float.....    | 63.3                  | 34.8                            | 4.53             | 15.6               | 43.7                            | 59.4             |
| Nonfloat..... | 36.7                  | 77.2                            | 12.3             | 3.43               | 56.3                            | 40.6             |

by screening at 65 mesh and assaying 55.9% NaHCO<sub>3</sub>.

When corrected for residual salts from the brine, due to drying without washing off the residual brine, the following results were achieved:

| Weight (%)    | Chemical analysis (%) |                                 |                  | Distribution (%)   |                                 |                  |
|---------------|-----------------------|---------------------------------|------------------|--------------------|---------------------------------|------------------|
|               | NaHCO <sub>3</sub>    | Na <sub>2</sub> CO <sub>3</sub> | SiO <sub>2</sub> | NaHCO <sub>3</sub> | Na <sub>2</sub> CO <sub>3</sub> | SiO <sub>2</sub> |
| Float.....    | 63.5                  | 36.7                            | 4.76             | 16.7               | 43.6                            | 58.7             |
| Nonfloat..... | 36.5                  | 82.8                            | 5.84             | 3.7                | 56.4                            | 41.3             |

In another test a sample of the same flotation feed as above was conditioned for 3 minutes with 0.25lb/ton flotation feed of Aeromine 3037 (cationic collector, 1 part dissolved in 3 parts of kerosine) and the gangue minerals were floated from Nahcolite:

| Weight (%)    | Chemical analysis (%) |                                 |                  | Distribution (%)   |                                 |                  |
|---------------|-----------------------|---------------------------------|------------------|--------------------|---------------------------------|------------------|
|               | NaHCO <sub>3</sub>    | Na <sub>2</sub> CO <sub>3</sub> | SiO <sub>2</sub> | NaHCO <sub>3</sub> | Na <sub>2</sub> CO <sub>3</sub> | SiO <sub>2</sub> |
| Float.....    | 59.6                  | 27.2                            | 11.5             | 16.5               | 35.4                            | 48.0             |
| Nonfloat..... | 40.4                  | 73.3                            | 18.4             | 3.0                | 64.6                            | 52.0             |
| Float.....    | 60.2                  | 28.5                            | 6.4              | 17.5               | 35.3                            | 46.1             |
| Nonfloat..... | 39.8                  | 79.5                            | 11.4             | 3.27               | 64.7                            | 53.9             |

The above tests were conducted at 71°F. and 93 percent relative humidity. The pump contained 17 percent solids and its pH was 10.2. The pH of the pulp may and 50 will possibly change depending on the constituents of the ore, their solubility and types of reagents used in flotation.

The foregoing results show single stage flotation. Scavenger flotation of the rougher tailing, that is float product, and a cleaner flotation of the rougher concentrate will increase the recovery and improve the grade of the concentrate. Scavenger flotation consists of re-floating the rougher float product, and additional Nahcolite will remain in the nonfloat product in that flotation. A cleaner flotation will include the flotation of the rougher underflow to remove the insoluble minerals such as quartz and calcite. Since the ores of the Nahcolite vary from location to location, the type and amount of reagent will change.

Possible application as collectors for the mentioned system of minerals i.e. Nahcolite ores may find a number of cationic collectors.

Important role in the flotation process could be played by alcohols as froth controlling agents. They

#### SAMPLE A

| Weight %      | Chemical Analysis % | Oil gal/ton        | Distribution %     |
|---------------|---------------------|--------------------|--------------------|
| Head (Calc'd) | NaHCO <sub>3</sub>  | NaHCO <sub>3</sub> | NaHCO <sub>3</sub> |
| Head (Calc'd) | 100.0               | 56.5               | 100.0              |
| Float         | 37.8                | 27.4               | 15.8               |
| Nonfloat      | 62.2                | 74.1               | 2.6                |

#### SAMPLE B

| Weight %      | Chemical Analysis % | Oil gal/ton        | Distribution %     |
|---------------|---------------------|--------------------|--------------------|
| Head (Calc'd) | NaHCO <sub>3</sub>  | NaHCO <sub>3</sub> | NaHCO <sub>3</sub> |
| Head (Calc'd) | 100.0               | 52.7               | 13.7               |
| Float         | 33.6                | 19.8               | 27.1               |
| Nonfloat      | 66.4                | 69.3               | 6.9                |

#### SAMPLE C

| Weight %      | Chemical Analysis % | Oil gal/ton        | Distribution %     |
|---------------|---------------------|--------------------|--------------------|
| Head (Calc'd) | NaHCO <sub>3</sub>  | NaHCO <sub>3</sub> | NaHCO <sub>3</sub> |
| Head (Calc'd) | 100.0               | 54.9               | 17.9               |
| Float         | 25.3                | 13.1               | 40.9               |
| Nonfloat      | 74.7                | 69.1               | 10.1               |

We claim:

1. A method of concentrating naturally occurring crystalline mineral Nahcolite from ores containing said Nahcolite and kerogen-bearing rock (oil shale), comprising the steps of:
  - a. crushing a portion of said ore;
  - b. collecting particles of crushed ore as an undersize fraction a substantial portion of which is below about 28 mesh in size;
  - c. said crushing being maintained in a manner to inhibit substantial smearing of oil from said rock on said undersize particles;
  - d. pulping said undersize particles in a brine in equilibrium with the soluble constituents in said ore to produce a flotation pulp;
  - e. aerating said pulped particles in said brine to produce a flotation froth;

- f. maintaining said pulping and aeration to effect a relative concentration of said rock in a first float portion in said froth, and said Nahcolite in a second non-float underflow portion;
  - g. separately withdrawing said float portion from said non-float underflow portion, thereby to effect a fractionation and separation of Nahcolite from said ore.
2. A concentration method as in claim 1 which includes the added step of conditioning said pulp by addition of an organic cationic collection agent selected from an organic amine and an organic amine salt.

3. A concentration method as in claim 1 which includes the step of adding 1-hexanol to said brine to control the frothing of said flotation pulp.

4. A concentration method as in claim 1 wherein said crushing is maintained in a hammer mill to inhibit substantial oil smearing.

5. A concentration method as in claim 1 wherein said kerogen-bearing rock contains less than about 41 gal/ton hydrocarbon-type oil.

6. A concentration method as in claim 1 wherein said 10 undersize fraction is below about 65 mesh in size.

\* \* \* \* \*

15

20

25

30

35

40

45

50

55

60

65